

Feb. 19, 1935.

K. W. YOUNG

1,992,049

ROASTING OF PLUMBIFEROUS PYRITES

Filed Jan. 20, 1933



INVENTOR.  
KENNETH WILLIAM YOUNG

BY *George Leeg*

ATTORNEY.

## UNITED STATES PATENT OFFICE

1,992,049

## ROASTING OF PLUMBIFEROUS PYRITES

Kenneth William Young, Norton-on-Tees, England, assignor to Imperial Chemical Industries Limited, a corporation of Great Britain

Application January 20, 1933, Serial No. 652,773  
In Great Britain January 23, 1932

5 Claims. (Cl. 23—134)

This invention relates to processes for roasting or burning sulphide ores such as pyrites which contain small amounts (up to about 5 per cent) of lead compounds, chiefly lead sulphide, for the purpose of recovering lead in a convenient manner.

When pyrites containing lead is burnt with air in a pyrites burner in the ordinary manner, the greater part of the lead is oxidized and remains with the burnt ore as lead oxide and other lead compounds.

I have found that pyrites containing lead, with or without other non-ferrous metals, may advantageously be treated for the production of sulphur and/or sulphur dioxide together with iron oxide, with the simultaneous volatilization of substantially the whole of the lead in the form of lead sulphide. The lead sulphide may then be separated from the roasting gases by suitable reduction of temperature and collection of the lead sulphide fume in suitable apparatus.

According to the invention, sulphide ores such as pyrites containing small amounts of lead are subjected to roasting with a limited supply of air or oxygen-containing gases in a rotary or shaft kiln or mechanical furnace so that the whole of the oxygen is used up and a portion of the heated material is in contact with gas free from oxygen. At the same time a stream of gas substantially free from oxygen, such as nitrogen or sulphur dioxide or a mixture of these, is introduced into the furnace at a suitable point, or points, preferably in the combustion zone, whereby lead sulphide is volatilized and carried off in the stream of gases.

The temperature of the combustion zone in the furnace should be carefully controlled so that the combustion gases at a point, immediately above the combustion zone, at which they no longer contain oxygen are at a sufficiently high temperature to volatilize the lead sulphide, whilst at the same time the temperature of the melting-point of the sulphide ore under treatment is not exceeded. Suitable temperatures are 800—900° C. I have found that with pyrites containing up to 5 per cent. of lead substantially the whole of the lead is volatilized at temperatures of 800—850° C.

The vapour pressure of lead sulphide at the temperatures employed is only small and it is therefore necessary to supply considerable quantities of gas, especially when the lead content of the sulphide ore is comparatively high. In general I have found that the quantity of inert gas should be about twice that of the combustion air

or gas and the rate of passage of the gas through the burner should be about 20 centimetres per second.

The absence of appreciable quantities of free oxygen in the zone where volatilization of the lead takes place is essential in order to avoid the combustion of lead sulphide to lead oxide. In the case of an ore or material containing such pyrites this is insured by controlling the rate of air supply. For materials poorer in sulphur and also in general it may be desirable to add to the ore a small quantity of coke or other carbonaceous material in order to ensure the early removal of free oxygen. Under such circumstances some free sulphur may be present in the gas and this is a guarantee that the conditions are non-oxidizing. Such free sulphur may be collected from the gas by suitable means after removal of the lead sulphide.

The oxygen free gas may be introduced together with air or oxygen-containing gas into the lower part of the furnace, or part or the whole of it may be introduced directly into the combustion zone. The gas introduced may in addition be employed to control the temperature conditions in the manner described in British Patent No. 359,478. When the content of lead is relatively high, the amount of gas required to volatilize the lead sulphide and carry it through the cooler regions at the top of the burner is comparatively large and in such cases, owing to too great a cooling effect, it will be necessary to preheat the gas whether it is introduced into the lower part of the furnace or into the combustion zone. Similarly in the case of a minimum amount of air or oxygen being used for the combustion in order to obtain an increased quantity of free sulphur in the gases produced, a sufficiently high temperature to volatilize the lead sulphide may not be reached unless the introduced gases are pre-heated.

I have found that a very suitable method of carrying out the invention is to employ as oxygen-free gas a mixture of sulphur dioxide and nitrogen obtained from the top of the furnace. Thus the lead-containing sulphide ores are subjected to the treatment as described and the gases issuing from the top of the burner are suitably treated, e. g. by cooling, for the removal first of lead sulphide and then of sulphur, and the residual gases containing sulphur dioxide are returned, with or without preheating, either to the combustion zone or partly to the combustion zone and partly to the lower part of the burner where they are mixed with the air or oxygen-containing gas.

The attached drawing shows a diagrammatic flow sheet of the process of this invention.

*Example*

5 In the treatment of a pyrites containing 2 per cent of lead and 45 per cent of sulphur the process may be carried out as follows:—

The pyrites in coarsely ground form is mixed with 10 per cent of its weight of powdered coke 10 and the mixture is fed continuously into the upper end of a rotary kiln at the rate of 100 kg. per hour. Air is blown into the lower end of the kiln at a rate corresponding to 130 cubic metres per 100 kg. of the pyrites. At a point above one third 15 the length of the kiln from the lower end a mixture of  $N_2$  and  $SO_2$  is introduced at such a rate that the maximum temperature in the kiln does not exceed 900° C. This gas is introduced at a 20 temperature of 200° C. and from 200 to 300 cubic metres per 100 kg. of pyrites will be required according to the rate of heat loss from the kiln. Under these conditions the pyrites is subjected to 25 strongly reducing conditions in the upper end of the kiln and the exit-gas consists of a mixture of  $N_2$ ,  $SO_2$ , sulphur vapour and  $CO_2$ , together with the vapour of lead sulphide. The gas is cooled to about 400° C. and passed through an electrostatic dust precipitator. Here a dust is collected which is rich in lead sulphide and which may be disposed 30 of or worked up for the recovery of lead in any known manner. The residual gas after complete cooling to condense the sulphur vapour is concentrated in  $SO_2$  and then returned to the pyrites burner. In the concentration sufficient nitrogen 35 is purged to correspond to the nitrogen contained in the air introduced into the burner.

The process according to the invention may advantageously be combined with the process for the sulphatization of zinc and copper in sulphide ores described in my co-pending British application No. 34770/31 issued as Patent No. 395,760. Thus in the combined process the sulphur dioxide containing gases issuing from the upper portion of the burner may be enriched in 40 sulphur dioxide in any desired manner and recirculated, a sufficient quantity of gas being passed through the burner or the upper part of it to volatilize the lead sulphide. If the temperature of the combustion zone is kept sufficiently high, i. e. not 45 lower than 850° C., and the velocity and quantity of the gas are sufficiently great (depending upon the quantity of lead contained in the ore) substantially the whole of the lead will be removed as lead sulphide in the issuing gases.

50 The treatment of the ore may also be carried out so as to effect the recovery of the sulphur in

the free state. For this purpose the conditions of roasting are strongly reducing and free carbon may be added in suitable form to assist in the reduction of sulphur dioxide to free sulphur. In general the methods described in British Patent No. 359,478 and in co-pending British application No. 2879/31 issued as Patent No. 391,136 may be employed, with such modifications as are described above to ensure the complete volatilization of the lead. 10

I claim:—

1. A process for the recovery of lead sulphide from iron sulphide ores containing small amounts of lead, which comprises roasting said ore with a limited supply of air so that the whole of the oxygen is used up in oxidizing the iron sulphide and a portion of the heated material is in contact with gas free from oxygen, introducing a stream of gas substantially free from oxygen in sufficient quantity and at a sufficient velocity and maintained at a sufficient temperature to volatilize substantially the whole of the lead sulphide and remove it in the form of vapour, cooling the exit gases and collecting the precipitated lead sulphide. 15

2. In a process of roasting an iron sulfide ore containing a small amount of lead sulfide for the recovery of the sulfur contained therein and the production of a cinder substantially free from lead the steps of feeding said ore into one end of an ore roasting furnace, introducing a first gas containing free oxygen into the other end of said furnace in an amount not exceeding that required to burn all the iron sulfide into iron oxide and sulfur dioxide, moving said ore in counter current to said gas, establishing a zone in said furnace near the entrance of said ore in which the unroasted ore is maintained at a temperature of about 800 to 900° C. and in which the gases in contact with the ore are substantially non-oxidizing, introducing into said furnace a second stream of gas which is free from oxygen, the amount of said second gas being at least about twice that of the first gas stream and maintaining the gas flow through said furnace at a rate of at least about 20 centimeters per second. 30

3. The process of claim 2 in which the gas stream leaving the furnace is treated to precipitate and recover the volatilized lead sulfide contained therein. 40

4. The process of claim 2 in which a solid carbonaceous material is mixed with the ore fed into the furnace. 45

5. The process of claim 2 in which the second gas stream is preheated. 50

KENNETH WILLIAM YOUNG.

**CERTIFICATE OF CORRECTION.**

**Patent No. 1,992,049.**

**February 19, 1935.**

**KENNETH WILLIAM YOUNG.**

It is hereby certified that error appears in the printed specification of the above numbered patent requiring correction as follows: Page 1, second column, line 8, for "such" read much; page 2, first column, line 14, for "above" read about; and second column, line 7, for "2879/31" read 28729/31; and that the said Letters Patent should be read with these corrections therein that the same may conform to the record of the case in the Patent Office.

Signed and sealed this 11th day of June, A. D. 1935.

(Seal)

**Leslie Frazer**  
**Acting Commissioner of Patents.**